

# United States Patent

[11] 3,615,530

[72] Inventors **Haruhiko Iwano;**  
**Isao Shimamura, both of Ashigarakamigun, Kanagawa, Japan**  
[21] Appl. No. **764,591**  
[22] Filed **Oct. 2, 1968**  
[45] Patented **Oct. 26, 1971**  
[73] Assignee **Fuji Shashin Film Kabushiki Kaisha**  
[32] Priority **Oct. 2, 1967**  
[33] **Japan**  
[31] **42/63359**

2,857,276 10/1958 Land et al. .... 96/66 X  
3,386,831 6/1968 Honig et al. .... 96/109  
2,311,098 2/1943 Swan et al. .... 96/109 X

Primary Examiner—William D. Martin  
Assistant Examiner—M. R. Lusignan  
Attorney—Sughrue, Rothwell, Mion, Zinn and MacPeak

[54] **PHOTOGRAPHIC PROCESS FOR  
PHOTOGRAPHIC SILVER HALIDE LIGHT-  
SENSITIVE ELEMENTS**  
2 Claims, No Drawings

[52] U.S. Cl. .... **96/66.5,**  
96/50 PT, 96/109  
[51] Int. Cl. .... **G03c 5/30,**  
G03c 5/38  
[50] Field of Search. .... **96/66.5,**  
109, 22, 50, 50 PT

[56] **References Cited**  
UNITED STATES PATENTS

|           |         |                      |          |
|-----------|---------|----------------------|----------|
| 1,763,989 | 6/1930  | Sheppard et al. .... | 96/109   |
| 2,184,023 | 12/1939 | Sheppard et al. .... | 96/109   |
| 2,319,090 | 5/1943  | Sheppard et al. .... | 96/109   |
| 2,354,662 | 8/1944  | Bryce ....           | 117/156  |
| 2,697,100 | 12/1954 | Knott ....           | 96/109 X |
| 2,857,274 | 10/1958 | Land et al. ....     | 96/66 X  |

**ABSTRACT:** An improved developing process for photographic silver halide elements wherein the element is subjected to processing between a prehardening step and a development step with an aqueous solution containing a heterocyclic compound having structural units which comprise at least two members which are from the group consisting of



at least one structural unit must be from the group consisting of



R<sub>1</sub>, R<sub>2</sub> and R<sub>3</sub> may each be a hydrogen atom, a methyl group or an ethyl group.

## PHOTOGRAPHIC PROCESS FOR PHOTOGRAPHIC SILVER HALIDE LIGHT-SENSITIVE ELEMENTS

### BACKGROUND OF THE INVENTION

#### 1. Field of the Invention

The present invention relates generally to a development process for photographic silver halide light-sensitive elements and more particularly to a process of reducing the formation of fogs caused by the hardening of silver halide emulsion layers of photographic silver halide light-sensitive elements.

#### 2. Description of the Prior Art

In general, when photographic light-sensitive films, printing papers, or photographic light-sensitive plates having silver halide are subjected to photographic processing, they are processed in a hardening bath prior to a development step.

The object of the hardening processing is to prevent the silver halide emulsion layers from being damaged mechanically or physically during the development process by increasing the mechanical or physical strength of the emulsion layers. In particular, the application of the hardening bath is very effective when silver halide emulsion layers do not originally have sufficient strength, the emulsion layers are to be processed for a long period of time, or the emulsion layers are to be processed in a solution having either a high temperature or a high pH. The hardening processing used prior to development is usually called "prehardening," and as a prehardening bath, there is usually employed an aqueous solution containing an aldehyde capable of hardening the gelatin in the photographic emulsion layer by the reaction therewith, such as, formaldehyde, glyoxal, succinaldehyde, glutaraldehyde, etc.

Although the use of such a prehardening bath effectively hardens photographic emulsion layers, it gives a bad influence on photographic properties, for example, the formation of development fogs is increased, the development density at reversal development is reduced, and the coupling property of couplers in photographic light-sensitive color elements is varied.

### SUMMARY OF THE INVENTION

It has been found that the formation of fogs caused by the hardening of silver halide emulsion layers in photographic light-sensitive elements may be reduced in a processing scheme wherein a prehardening step and a development step is utilized by subjecting the element to a processing step between prehardening and development which comprises subjecting the element to an aqueous solution containing a heterocyclic compound having structural units which comprise at least two members which are from the group consisting of



At least one of the structural units must be from the group consisting of



R<sub>1</sub>, R<sub>2</sub> and R<sub>3</sub> are selected from the group consisting of a hydrogen atom, a methyl group and an ethyl group.

The heterocyclic compound is generally utilized in a concentration of 0.1-50 g./liter.

Thus, an object of the present invention is to provide an improved method of processing photographic silver halide light-sensitive elements which provides good photographic properties and sufficient mechanical strength to photographic emulsion layers, without any of the faults known in the prior art.

### DESCRIPTION OF THE PREFERRED EMBODIMENTS

According to the process of the present invention, photographic silver halide emulsion layers are processed between prehardening processing and development processing in an aqueous solution containing a heterocyclic compound (including a tautomer thereof) having as structural units at least two of the groups:



(at least one of which



wherein R<sub>1</sub>, R<sub>2</sub> and R<sub>3</sub> may represent a hydrogen atom, a methyl group or an ethyl group.

Typical examples of such compounds are maleic hydrazide, dimedone, uracil, cyanuric acid, succinimide, flavanic acid, barbituric acid, and melamine.

By using the aforesaid heterocyclic compound, generally in a concentration of 0.1-50 g./liter, the aldehyde remaining after hardening processing is effectively removed, whereby the entrance of the aldehyde in the subsequent processing step is effectively prevented.

The aqueous solution for antifogging processing is preferred and may be used at any pH, but better results can be obtained when it is used in a neutral or acid state. Moreover, the aqueous solution containing the aforesaid heterocyclic compound may further contain pH-controlling agents and buffering agents, such as sodium sulfate, borax, acetic acid, sodium acetate, sodium carbonate, sulfuric acid, boric acid, etc., and also other general antifogging agents, such as an alkali halide.

The light-sensitive emulsion layer to be processed by the process of this invention contains, as a light-sensitive material, a conventionally-employed silver halide, and as a dispersoid for the light-sensitive material, gelatin or a mixture of gelatin and another hydrophilic high molecular weight material. Supports for the photographic emulsion layers may be glass plates, cellulose ester films, polyester films, and papers. These are commonly used in the photographic art.

The process of this invention may most suitably be applied to the case of processing light-sensitive reversal color elements which are processed at a high pH or for a long period of time; it is also particularly applicable to color photographic printing papers which are preferably quickly processed at high temperature.

In the practice of the process of this invention, a photographic light-sensitive element is, after being subjected to prehardening processing, processed in the antifogging bath of this invention, and thereafter subjected to conventional subsequent processings, including development.

By the process of the present invention, the formation of development fogs is lessened, reduction in development density does not occur, and the coupling property of couplers in light-sensitive color elements is not varied.

The following examples will further explain the process of this invention in detail, although the invention is not limited to them.

### EXAMPLE 1

A black and white negative photographic light-sensitive film prepared by applying a gelatino silveriodobromide emulsion sufficiently panchromatically color sensitized was exposed by means of a sensitometer and subjected to the following photographic processings at 40° C.:

| Processing             | Time    |
|------------------------|---------|
| Prehardening           | 35 sec. |
| Washing                | 10 sec. |
| Antifogging processing | 45 sec. |
| Washing                | 20 sec. |
| Development            | 50 sec. |

|          |         |
|----------|---------|
| Stopping | 10 sec. |
| Fixing   | 30 sec. |
| Washing  | 90 sec. |

The compositions of the processing solutions used in the above processings are as follows:

**Prehardening composition:**

|                          |          |
|--------------------------|----------|
| Sodium bisulfite         | 1 g.     |
| Formalin (37% aq. soln.) | 15 ml.   |
| Borax                    | 5 g.     |
| Sodium sulfate           | 50 g.    |
| Potassium bromide        | 2 g.     |
| Water to make            | 1 liter. |

**Antifogging composition:**

The heterocyclic compound shown in the following table was dissolved in 1 liter of an aqueous solution containing 5 g. of glacial acetic acid and 4 g. of sodium acetate to provide seven different embodiments of the antifogging baths of this invention. A control solution which did not contain the heterocyclic compound of this invention was also prepared.

| Test No. | Additive         | Amount |
|----------|------------------|--------|
| 1        | none             |        |
| 2        | maleic hydrazide | 2 g.   |
| 3        | dimedone         | 2 g.   |
| 4        | uracil           | 3 g.   |
| 5        | cyanuric acid    | 5 g.   |
| 6        | succinimide      | 5 g.   |
| 7        | flavanic acid    | 5 g.   |
| 8        | barbituric acid  | 5 g.   |

  

| Developer:                   |         |      |
|------------------------------|---------|------|
|                              | Metol   | 5 g. |
| Hydroquinone                 | 2 g.    |      |
| Sodium sulfite               | 70 g.   |      |
| Sodium hydroxide             | 1 g.    |      |
| Sodium carbonate monohydrate | 41 g.   |      |
| Potassium bromide            | 2 g.    |      |
| Water to make                | 1 liter | g.   |

  

| Stopping composition: |                     |         |
|-----------------------|---------------------|---------|
|                       | Glacial acetic acid | 15 ml.  |
| Water to make         |                     | 1 liter |

  

| Fixing composition: |                    |        |
|---------------------|--------------------|--------|
|                     | Sodium thiosulfate | 150 g. |
| Sodium sulfite      | 15 g.              |        |
| Water to make       | 1 liter            |        |

The results of the photographic processings are shown in table 1, in which the relative sensitivity is shown by the logarithmic value of a reciprocal of the exposure amount corresponding to the blackened density of a 0.1 over fog.

TABLE 1

| Test No.          | Fog  | Relative Sensitivity |      |
|-------------------|------|----------------------|------|
| Gamma Value       |      |                      |      |
| 1 (control)       | 0.36 | 2.20                 | 0.32 |
| 2                 | 0.23 | 2.35                 | 0.37 |
| 3                 | 0.25 | 2.33                 | 0.36 |
| 4                 | 0.22 | 2.36                 | 0.36 |
| 5                 | 0.24 | 2.33 tm 0.35         |      |
| 6                 | 0.25 | 2.35                 | 0.35 |
| 7                 | 0.25 | 2.32                 | 0.35 |
| 8                 | 0.24 | 2.34                 | 0.36 |
| No bath (control) | 0.37 | 2.20                 | 0.31 |

PS

It is clear from the results shown in the above table that by the application of the antifogging bath of this invention, the formation of development fogs was effectively prevented and the sensitivity and the gamma value were increased.

In addition, the application of the antifogging bath enables the practice of prehardening processing whereby the mechani-

70

cal strength of the photographic emulsion layer is increased, and hence high-temperature processing can be applied without being accompanied by operational problems.

## EXAMPLE 2

A photographic gelatino silver halide emulsion layer (panchromatically color-sensitized and applied to a polyester film) was exposed through a silver step wedge by means of a sensitometer and subjected to the following photographic processings at 27°C.:

|    | Process                | Time     |
|----|------------------------|----------|
| 15 | Prehardening           | 60 sec.  |
| 10 | Washing                | 30 sec.  |
| 20 | Antifogging processing | 60 sec.  |
|    | Washing                | 30 sec.  |
|    | Primary development    | 210 sec. |
|    | Washing                | 30 sec.  |
|    | Bleaching              | 180 sec. |
|    | Washing                | 30 sec.  |
|    | Cleaning               | 60 sec.  |
|    | Washing                | 30 SEC.  |
| 25 | Second development     | 120 sec. |
|    | Washing                | sec. 30  |
|    | Fixing                 | 90 sec.  |
|    | Washing                | 150 sec. |
|    | Drying                 | 180 sec. |

In the above processings, only drying was conducted at 38° C. The compositions of the processing solutions used in the above processings are as follows:

**Prehardening composition:**

Same as in example 1.

**Antifogging composition**

The heterocyclic compound shown in the following table was added to 1 liter of an aqueous solution containing 4 g. of sodium acetate, 5 ml. of glacial acetic acid, and 0.7 g. of potassium bromide.

| Test No. | Additive         | Amount |
|----------|------------------|--------|
| 1        | none             |        |
| 2        | maleic hydrazide | 2 g.   |
| 3        | dimedone         | 2 g.   |
| 4        | uracil           | 3 g.   |
| 5        | cyanuric acid    | 5 g.   |

**Primary and secondary developers:**

0.8 g./liter of potassium thiocyanate was added to the developer in example 1.

**Bleaching solution:**

|                      |         |
|----------------------|---------|
| Sulfuric acid        | 5 ml.   |
| Potassium bichromate | 5 g.    |
| Water to make        | 1 liter |

**Cleaning composition:**

|                |         |
|----------------|---------|
| Sodium sulfite | 50 g.   |
| Water to make  | 1 liter |

**Fixing composition:**

Same as in example 1.

The results are shown in table 2.

TABLE 2

| Test No.    | Reversal density |
|-------------|------------------|
| 1 (control) | 1.12             |
| 2           | 1.52             |
| 3           | 1.50             |
| 4           | 1.55             |
| 5           | 1.48             |

It is clear from the above results that since the reversal density was increased by the use of the antifogging bath of this invention, good photographic properties were obtained while employing the prehardening processing. Furthermore, by the process of this invention the surface of the photographic emulsion layer was prevented from being damaged mechanically during processing and the drying load for the photographic film was reduced.

## EXAMPLE 3

A multiple layer photographic color film prepared by applying to a cellulose acetate film a gelatino silver iodobromide emulsion having a red sensitivity, a gelatino silver iodobromide emulsion having a green sensitivity, a yellow filter layer containing fine colloidal silver particles and have a blue-absorptive property, and a gelatino silver iodobromide emulsion having a blue sensitivity (in this order) and exposed through a silver step wedge by means of a sensitometer was subjected to the following processings at 24° C.:

| Processing             | Time   |
|------------------------|--------|
| Prehardening           | 1 min. |
| Washing                | 1 min. |
| Antifogging processing | 1 min. |
| Washing                | 1 min. |
| Primary development    | 5 min. |
| Washing                | 2 min. |

Reversal exposure (red light) 200CMS from the back side of the film.

| Cyan color development | 5 min. |
|------------------------|--------|
| Washing                | 2 min. |

Reversal exposure (blue light) 200 CMS from the emulsion layer side of the film.

| Yellow color development | 5 min. |
|--------------------------|--------|
| Washing                  | 1 min. |
| Secondary development    | 1 min. |
| Washing                  | 1 min. |

Reversal exposure (white light) 2000 CMS from the opposite sides of the film.

| Magenta color developer | 5 min. |
|-------------------------|--------|
| Washing                 | 5 min. |
| Bleaching               | 2 min. |
| Washing                 | 1 min. |
| Fixing                  | 2 min. |
| Washing                 | 2 min. |

The compositions for the above processings are as follows:

Prehardening composition:

Same as in example 1.

Antifogging composition:

The heterocyclic compound shown in the following table was added to 1liter of an aqueous solution containing 8 g. of boric acid, 0.3 ml. of sulfuric acid and 0.8 g. of potassium bromide.

| Test No.    | Additive         | Amount |
|-------------|------------------|--------|
| 1 (control) | none             |        |
| 2           | maleic hydrazide | 2 g.   |
| 3           | dimedone         | 2 g.   |
| 4           | uracil           | 3 g.   |
| 5           | cyanuric acid    | 5 g.   |
| 6           | succinimide      | 5 g.   |
| 7           | flavanic acid    | 5 g.   |
| 8           | barbituric acid  | 2 g.   |

Primary and secondary black and white developer:

Same as in Example 2.

Cyan color developer:

Sodium sulfite

|                                       |         |
|---------------------------------------|---------|
| 2-Amino-5-diethylaminotoluene sulfate | 0.6 g.  |
| Sodium carbonate monohydrate          | 15.0 g. |
| Potassium bromide                     | 0.5 g.  |
| Potassium iodide (0.1% aq. soln.)     | 5.0 ml. |
| 1,5-Dihydroxy-2,6-dibromonaphthalene  | 1.2 g.  |
| Sodium hydroxide                      | 2.0 g.  |
| Water to make                         | 1 liter |

|                                                |         |
|------------------------------------------------|---------|
| Yellow color developer:                        |         |
| Sodium sulfite                                 | 5.0 g.  |
| N,N-Diethyl-p-phenylenediamine sulfite         | 2.5 g.  |
| Potassium bromide                              | 1.0 g.  |
| Potassium iodide (0.1% aq. soln.)              | 5.0 ml. |
| o-Benzoyl-4-p-(toluenesulfonamide)-acetanilide | 1.2 g.  |
| Sodium hydroxide                               | 2.5 g.  |
| Water to make                                  | 1 liter |

|                                             |         |
|---------------------------------------------|---------|
| Magenta color developer:                    |         |
| Sodium sulfite                              | 5.0 g.  |
| 2-Amino-5-diethylaminotoluene hydrochloride | 2.0 g.  |
| Potassium bromide                           | 0.8 g.  |
| 1-Phenyl-3-(m-nitrobenzoylamo)-5-pyrazolone | 1.4 g.  |
| Sodium hydroxide                            | 2.0 g.  |
| n-Butylamine                                | 5.0 g.  |
| Water to make                               | 1 liter |

|                        |           |
|------------------------|-----------|
| Bleaching solution:    |           |
| Potassium ferricyanide | 100 t. g. |
| Potassium bromide      | 20 g.     |
| Borax                  | 2.0 g.    |
| Boric acid             | 1.0 g.    |
| Water to make          | 1 liter   |

|                    |         |
|--------------------|---------|
| Fixing solution:   |         |
| Sodium thiosulfate | 150 g.  |
| Sodium sulfite     | 10 g.   |
| Water to make      | 1 liter |

The photographic characteristics (reversal coupling density) thus obtained are shown in the following table.

TABLE 3

| Test No. | Reversal density |               |              |
|----------|------------------|---------------|--------------|
|          | Red density      | Green density | Blue density |
| 40       |                  |               |              |
| 45       | 1 3.05           | 2.95          | 2.90         |
|          | 2 3.43           | 3.40          | 3.44         |
|          | 3 3.47           | 3.42          | 3.46         |
|          | 4 3.48           | 3.38          | 3.47         |
|          | 5 3.42           | 3.40          | 3.42         |
|          | 6 3.44           | 3.42          | 3.42         |
|          | 7 3.44           | 3.40          | 3.40         |
| 50       | 8 3.43           | 3.41          | 3.41         |

From the results, it is confirmed that the coupling densities were remarkably increased by the antifogging processing of this invention. Furthermore, contamination, decrease in sensitivity and other harmful influences on the photographic properties of the film were not observed.

## EXAMPLE 4

60 A commercially available color photographic printing paper was exposed by means of a sensitometer and then processed as follows at 20° C. (except drying, which was conducted at 38° C.)

|    |                      |         |
|----|----------------------|---------|
| 65 | Processing I         | Time    |
|    | Color development    | 5 min.  |
|    | Washing              | 5 min.  |
|    | Bleach-fixing        | 8 min.  |
|    | Washing              | 10 min. |
|    | Hardening            | 5 min.  |
|    | Buffering processing | 5 min.  |
|    | Washing              | 5 min.  |
|    | Stabilization        | 5 min.  |
|    | Drying               | 5 min.  |

70 The compositions used in the above processings are as follows:

Primary and secondary black and white developer:

Same as in Example 2.

Cyan color developer:

Sodium sulfite

5.0 g.

Color developer:  
 N-ethyl-n-hydroxyethyl-p-phenylene-diamine sulfate 7.5 g.  
 Hydroxylamine sulfate 0.3 g.  
 Potassium carbonate 100 g.  
 Potassium bromide 1 g.  
 Sodium sulfite (anhydrous) 4.5 g.  
 Sodium tripolyphosphate 1 g.  
 Water to make 1 liter

Bleach-fixing composition:  
 Iron salt of ethylenediamine-tetracetic acid 50 g.  
 Sodium carbonate (anhydrous) 2.5 g.  
 Sodium sulfite (anhydrous) 10 g.  
 Sodium thiosulfate (anhydrous) 200 g.  
 Water to make 1 liter

Hardening composition:  
 Tetrasodium salt of ethylene-diaminetetraacetic acid 0.5 g.  
 Sodium carbonate 10 g.  
 Sodium sulfate 50 g.  
 Formalin (37% aq. soln.) 50 ml.  
 Sodium bisulfite 4 g.  
 Water to make 1 liter

Buffering composition:  
 Tartaric acid 10 g.  
 Borax 25 g.  
 Water to make 1 liter

Stabilization composition:  
 Whitening agent (Tinopol; trade name, made by Geigy A.G.) 4 g.  
 Sodium dihydrogen phosphate 4 g.  
 Disodium hydrogen phosphate 2 g.  
 Tetrasodium salt of ethylene-diaminetetraacetic acid 1 g.  
 Water to make 1 liter

Although good photographic qualities were obtained by the above processing, there was one fault and that was that exposed printing paper had to be processed for a longer period of time. Thus, to reduce the processing time, the whole processing was conducted at 35°C. (processing II.) However, a so-called reticulation was formed on the emulsion layer, and this reduced the commercial value of the printing paper.

To obviate this, the hardening step was carried out prior to the color development step (processing III.) That is, the hardening process in processing I was omitted, and as a substitute, therefore the printing paper was processed for 60 seconds before the color development in a hardening solution having the following composition:

Hardening composition:  
 Formalin (37% aq. soln.) 20 ml.  
 2,5-dimethoxytetrahydrofuran 4 ml.  
 Sulfuric acid 2 ml.  
 Sodium sulfate 100 g.  
 Potassium bromide 2 g.  
 Borax 5 g.  
 Water to make 1 liter

By this processing, the mechanical strength of the light-sensitive emulsion layer of the printing paper was sufficiently increased, but development fogs were severely formed by processing III. This also reduced the commercial value of the printing paper, the same as in processing II.

However, when the printing paper was subjected to the processings of this invention (after exposure) employing antifogging processing (processing IV.) good photographic qualities as in the standard processing (processing I) were obtained, and the processing time was shortened as shown below while maintaining sufficient mechanical strength of the photographic emulsion layer of the printing paper during processing. The following processings were conducted at 38°C. (except drying, which was conducted at 50°C.)

Processing IV  
 Hardening 60 sec.  
 Washing 30 sec.  
 Antifogging processing 60 sec.

washing 30 sec.  
 Color development 100 sec.  
 Washing 30 sec.  
 Bleach-fixing 140 sec.  
 Washing 30 sec.  
 Buffering processing 40 sec.  
 Washing 30 sec.  
 Stabilization 40 sec.  
 Drying

10 The composition for the antifogging processing was an aqueous solution containing 3 g./liter of uracil and 0.5 g./liter of potassium bromide. The composition for the hardening processing was the same as in processing III.

15 The fogging densities of the color printing papers obtained by processings I, II, III, and IV are shown in the following table.

TABLE 4

| Processing | Red density | Fog Density   |              |
|------------|-------------|---------------|--------------|
|            |             | Green density | Blue density |
| I          | 0.08        | 0.08          | 0.11         |
| II         | t III       | 0.20          | 0.45         |
| IV         | 0.10        | 0.09          | 0.11         |

30

## EXAMPLE 5

35 A gelatino silver halide emulsion layer having a red sensitivity formed on a cellulose acetate film was exposed by means of a sensitometer through a silver step wedge and then subjected to the following reversal color processing at 24°C.:

| Processing: | Time     | Reversal exposure at 200 CMS. under white light. |         |                        |         |                     |         |
|-------------|----------|--------------------------------------------------|---------|------------------------|---------|---------------------|---------|
|             |          | Prehardening                                     | Washing | Antifogging processing | Washing | Primary development | Washing |
| 40          | 60 sec.  |                                                  |         |                        |         | 210 sec.            |         |
|             | 60 sec.  |                                                  |         |                        |         | 60 sec.             |         |
|             | 60 sec.  |                                                  |         |                        |         | 60 sec.             |         |
|             | 60 sec.  |                                                  |         |                        |         | 60 sec.             |         |
|             | 210 sec. |                                                  |         |                        |         | 60 sec.             |         |
|             | 60 sec.  |                                                  |         |                        |         | 60 sec.             |         |
|             | 60 sec.  |                                                  |         |                        |         | 60 sec.             |         |
|             | 60 sec.  |                                                  |         |                        |         | 60 sec.             |         |
|             | 60 sec.  |                                                  |         |                        |         | 60 sec.             |         |
|             | 60 sec.  |                                                  |         |                        |         | 60 sec.             |         |

30 The compositions for the prehardening and antifogging processings used above were the same as in example 1, the other compositions being the same as in example 3. The results are shown in the following table.

TABLE 5

| Additive | Amount                | Reversal density |  |
|----------|-----------------------|------------------|--|
|          |                       | (red density)    |  |
| 60       | none (control)        | 0.55             |  |
|          | Maleic hydrazide 2 g. | 0.98             |  |
|          | Dimedone 2 g.         | 1.05             |  |
|          | Uracil 5 g.           | 1.10             |  |
|          | Cyanuric acid 5 g.    | 1.07             |  |
|          | Succinimide 5 g.      | 1.03             |  |
|          | Flavanic acid 5 g.    | 0.99             |  |
|          | Barbituric acid 2 g.  | 0.96             |  |
|          | No bath (control)     | 0.55             |  |

70 By using the antifogging bath, the coupling density was remarkably increased, as shown in the above table.

## EXAMPLE 6

75 Reversal magenta color development was conducted basically as in example 5. Specifically, the cyan color developer in Example 5 was replaced with the magenta color developer in

example 3, and as the antifogging composition, the following solution was employed. However, the same basic procedure as in example 5 was repeated. The composition for the antifogging processing used in this example was an aqueous solution containing 50 g./liter of sodium sulfate, 5.0 g./liter of sodium bisulfite, 1.0 g./liter of borax, 0.5 g./liter of potassium bromide, and the heterocyclic compound shown in the following table.

| Test No. | Additive        | Amount (g./liter) |
|----------|-----------------|-------------------|
| 1        | none            |                   |
| 2        | Dimedone        | 4                 |
| 3        | Uracil          | 3                 |
| 4        | Cyanuric acid   | 5                 |
| 5        | Barbituric acid | 2                 |

The results are shown in the following table.

TABLE 6

| Test No.    | Reversal density |
|-------------|------------------|
| 1 (control) | 1.50             |
| 2           | 2.25             |
| 3           | 2.29             |
| 4           | 2.31             |
| 5           | 2.21             |

What is claimed is:

1. In a photographic processing method comprising pre-

hardening and developing a silver halide emulsion layer of a photographic silver halide light-sensitive element, the improvement which comprises processing said silver halide emulsion layer between said prehardening step and said development step in an acidic or neutral aqueous solution containing from about 0.1 to about 50 g./liter of said aqueous solution of a heterocyclic compound having structural units which comprise at least two members of the group consisting of:

10



at least one of said structural units being a member selected from the group consisting of:

20



wherein  $\text{R}_1$ ,  $\text{R}_2$  and  $\text{R}_3$  each represents a member selected from the group consisting of a hydrogen atom, a methyl group, and an ethyl group.

2. The photographic processing method as claimed in claim 1 wherein said heterocyclic compound is selected from the group consisting of hydrazide, dimedone, uracil, cyanuric acid, succinimide, flavanic acid, barbituric acid, and melamine.

\* \* \* \* \*

35

40

45

50

55

60

65

70

75